

Nov. 8, 1938.

G. S. HIERS

2,135,711

MANUFACTURE OF PILE FABRICS

Filed March 11, 1935



## UNITED STATES PATENT OFFICE

2,135,711

## MANUFACTURE OF PILE FABRICS

Glen S. Hiers, Bala-Cynwyd, Pa., assignor to Collins & Alkman Corporation, Philadelphia, Pa., a corporation of Delaware

Application March 11, 1935, Serial No. 10,405

2 Claims. (Cl. 91—68)

My invention relates to the manufacture of pile fabrics having V-pile tufts looped over the wefts of a loosely woven backing during the fabrication thereof and secured to such backing by the solidification therein of a solidifiable constituent of an aqueous material applied to the backing to form a layer or bed of binder in the backing.

My invention involves the elimination or minimizing of the effect of water-repellent substances contained in or on the yarns of the backing so as to facilitate and render more uniform the penetration of the aqueous material into the backing and the yarns of which it is composed, to prevent the formation of a skin coating of binder upon and separable from the backing or the yarns thereof, and to prevent absorption of oil or the like from the textile into the binder layer and thereby avoid the partial swelling of the layer of binder from such absorption. Such swelling tends to deleteriously reduce the tensile strength of the binder layer and to reduce the bond between it and the textile fibres. By my improvements, the tufts and backing yarns are more effectually secured relatively to one another with the use of a minimum amount of solidifiable impregnating material and without detracting from the textile characteristics of the product.

The water-repellent substances normally present in the fibres, and which tend to weaken the tensile strength and bond of a binder layer and to cause the formation of a surface skin, may be the natural waxes, oils, pectins or resins present in both animal and vegetable textile fibres or may be lubricants applied to such fibres in the spinning or processing thereof, and in accordance with my invention such waxes, oils, resins, pectins, lubricants or other water repellent substances may be removed from the yarns after or before the weaving thereof, and may be extracted or neutralized by solvents, absorbents, detergents, scouring, or reagents selected for their suitability for removing or rendering harmless the particular water-repellent substance or substances present in the fibres being treated.

When the water-repellent substances present in the fibres consist primarily of naturally present or applied oils, greases, waxes, pectins or resins, it is preferable to effect their removal, prior to impregnating the fabric, by scouring the yarns or the pile fabric woven therefrom with a detergent solution of soap, ammonia, soda or other alkali, or with suitable oil solvents, which may be of the chlorinated type or emulsified with water to avoid inflammability. During the treatment of the back of the fabric with the detergent or solvent,

the fabric may be subjected to brushing and the pressure of nip rolls to render the treatment more effective.

If the fibres used are naturally free from deleterious amounts of water-repellent substances, a water soluble lubricant, such as diethylene glycol or its homologues or derivatives, may be used in the preparatory process and spinning of the fibres and the oily lubricants generally used dispensed with. The removal of such water soluble lubricants may be effected by treatment of the yarns or fibres with water alone.

In some cases it is undesirable to wet the yarns or fibres with detergent or solvent substance, and in such cases the grease, oil and other water-repellent media may be removed and neutralized by the application to the back of the fabric of fuller's earth, other absorbent clays, or chemically treated silicate having high absorbent power. Such absorbents may be dusted on to the back of the fabric, brushed well into the interstices of the fabric, and then brushed off. Several applications may be made in this manner until a desired diminution of the content of water-repellent substance has been effected; and where animal and vegetable fibres containing different types of water-repellent substances are incorporated in the fabric or in the yarn from which it is made, such fabric or yarn may be subjected to such sequential treatments as are necessary to remove, neutralize or unify the effect of the several water-repellent substances contained in the different types of fibres and render more uniform the absorbent or permeable properties of the fibres.

When the water-repellent substances have been eliminated or reduced in amount to a desired degree from some or all of the yarns composing the fabric or from part of each of the elements of yarn composing the fabric and particularly those portions of the yarns contacting with the embedded binder layer, the fabric may be dried before impregnation, or may be impregnated while still wet, with an aqueous material containing a solidifiable constituent, such as latex, artificial aqueous dispersions of rubber, or synthetic rubber derived from chloroprene or aqueous dispersions of pyroxylin or other cellulose derivatives.

In the accompanying drawing, Fig. 1 illustrates diagrammatically an apparatus suitable for the practice of my invention, and Fig. 2 illustrates a second form of such apparatus. These apparatuses may be used in sequence or separately and both or either may constitute a unit in a range of plush dyeing and finishing equipment.

As illustrated in Fig. 1 of the drawing, a continuous strip of pile fabric A woven from yarns containing water-repellent substances and comprising a loosely woven backing with V-pile tufts 5 looped over the wefts thereof, is drawn face downward over the rollers 1, 2, 3 and 4 and beneath the rotary brush 5 which contacts with a fabric section suspended between the rollers 3 and 4 and applies to the back surface of such section a powdered or liquid remover or neutralizer for one or more of the hydrofuge substances contained in the yarn of which the backing and pile tufts are composed. Such remover or neutralizer may be supplied to the brush 5 at a desired rate through valved discharge ports 6 of a supply reservoir 7 above the brush. The remover or neutralizer is worked thoroughly into the fibres of the fabric by the rotation of the brush and any surface excess discharged from the fabric into a valved receiver 8. The brushed fabric may be then passed between rubber covered nip rolls 9 which apply pressure to the remover or neutralizer and force it into the fabric in intimate contact with the hydrofuge substances. Any free remover or neutralizer remaining after the passage of the fabric between the nip rolls may be removed by the suction extractor 10.

The fabric may then be passed, if desired, over a second set of rollers 3', 4', under the brush 5', 30 and treated with the same or a different remover or neutralizer supplied from the reservoir 7'. This second remover or neutralizer is brushed into the back of the fabric, the surplus discharged into the receiver 8' and the impregnated or embedded remover or neutralizer pressed into intimate contact with the hydrofuge substances by the nip rollers 9'. The free remover or neutralizer remaining after the second treatment is evacuated by the suction extractor 10'.

40 In lieu of or in addition to passage through one or more of the dehydrofuging devices shown in Fig. 1, the back of the fabric may be subjected to the action of scouring apparatus such as shown in Fig. 2. In this apparatus, an endless belt 100 is passed through a solvent or detergent emulsion contained in a tank 101 provided with guide rolls 102 and nip rolls 103 for translating the belt and squeezing excess liquid therefrom. The belt is guided over rolls 104, which may be rectilinearly 45 movable, into contact with a section of the back of the fabric A, which may be held flat or curved by card clothing rolls 105 and plain rolls 106.

The wet belt or apron 100 may be moved longitudinally in either direction, and if desired also 50 moved transversely, in contact with the back of the traveling fabric A, which is continuously scoured thereby. The extracted hydrofuge substances are gradually accumulated in the tank 101 and may be removed therefrom and the solvent or detergent liquid replenished as required.

When the hydrofuge substances have been sufficiently removed from the fabric by the treatment or treatments thereof as above described, the fabric may be then passed over the rollers 2' 55 and 1' and over the surfaces of the steam-heated drums 11 and 11' by which any volatile material may be driven off and the fabric dried, either wholly or partially. The passage of the fabric over the drums is controlled by the guides 12, 13, 60 14 and 15.

70 After drying, the fabric may have a normal or desired moisture content imparted to the back, in excess of that contained in the pile tufts, by passage of the fabric over guide rollers 16' and 75 through the steam box 16 with the pile face up-

ward and over steam jets 17. Any tufts which have been materially loosened by the treatment for the removal or neutralization of hydrofuge substances are brushed off by the brush 18, and slightly loosened tufts are forced back into position by the roller 19 and stationary cylinder 20 on opposite sides of the card clothing roller 21. The card clothing rollers 21 and 22 are provided with wire teeth which support the fabric backing without applying pressure to the cut ends of the 10 pile tufts.

In passing from the card clothing roller 21 to the card clothing roller 22, the fabric passes beneath a blade 23 to which the baffle plate 24 discharges a layer of uniform thickness of a hydro-sol, such as latex, containing a solidifiable constituent, and is discharged to the baffle plate through cocks 25 of an adjustable reservoir 26. The hydro-sol is forced into the interstices of the fabric by the action of the blade 23 and of the roller 21 so as to leave the bights of the pile tufts exposed to form a nodulous surface imparting to the fabric a textile "feel" and "handle." The hydro-sol permeates into the backing, without passing therethrough to the pile face of the fabric, and is solidified as a layer lying primarily in the backing by the passage of the fabric through a tenter drier 28 while stretched by the engagement of its selvages by the pins of tenter chains 29.

By the steps of removing or neutralizing water-repellent substances in the yarns, which for brevity in the claims I have called dehydrofuging the yarns, I am enabled to secure an intimate contact between the solidifiable constituent of a hydro-sol and the fibres of the fabric and avoid the formation of a surface skin on the yarns or fabric, and to improve the anchorage of the pile tufts to the backing and the backing yarns to one another, with consequent improvement in the durability 40 as well as in the appearance of the fabric, uses less rubber and so economies are effected, better tensiles and elasticities are produced due to absence of oil absorption, and better ageing results.

Having described my invention, I claim:

1. In the manufacture by a continuous process of an impregnated air permeable pile fabric having pile elements looped about wefts of a loosely woven backing, said pile elements originally containing water repellent bond inhibiting substances, the steps of removing or neutralizing the bond inhibiting substances by local application to the bights of the pile elements and the backing of an inorganic absorbent of such quality that it removes or neutralizes said inhibiting substances, passing the treated pile fabric adjacent to and substantially in contact with an air extractor employing a current of air which current passes through the fabric whereby portions of the bond inhibitor and remover are taken out of the pile fabric and the interstices of the fabric are left open, brushing the fabric to remove loose pile tufts and force slightly loosened pile tufts back into the fabric, depositing a uniform layer of a rubber hydro-sol on the back of said fabric, forcing the hydro-sol into the fabric, leaving the interstices of the fabric open and the bights of the pile exposed to form a nodulous surface imparting a textile feel and handle to the fabric, the quantity of hydro-sol being controlled so that it is substantially confined to the plane of the woven backing, and setting the hydro-sol whereby the pile is adhered to the backing.
2. In the manufacture by a continuous process

of an impregnated air permeable pile fabric having pile elements looped about wefts of a loosely woven backing, said pile elements originally containing water repellent bond inhibiting substances, the steps of removing or neutralizing the bond inhibiting substances by local application to the bights of the pile elements and the backing of an inorganic absorbent of such quality that it removes or neutralizes said inhibiting substances, 5 passing the treated pile fabric adjacent to and substantially in contact with an air extractor employing a current of air, which current passes through the fabric whereby portions of the bond 10 inhibitor and remover are taken out of the pile fabric and the interstices of the fabric are left open, depositing a uniform layer of a rubber hydrosol on the back of said fabric, forcing the hydrosol into the fabric, leaving the interstices of the fabric open and the bights of the pile exposed to form a nodulous surface imparting a textile feel and handle to the fabric, the quantity of hydrosol being controlled so that it is substantially confined to the plane of the woven backing, and 15 setting the hydrosol whereby the pile is adhered to the backing.

GLEN S. HIERS.